

Nov. 16, 1926.

1,607,118

C. L. DELACHAUX

METHOD OF AND APPARATUS FOR REPAIRING THE ENDS OF RAILS BY THE

ALUMINO-THERMIC PROCESS

Filed August 15, 1923

*Fig. 1*



*Fig. 2*



*Fig. 3*



INVENTOR

C. L. Delachaux

*Clas. & Name*  
HIS ATTORNEY

Patented Nov. 16, 1926.

1,607,118

# UNITED STATES PATENT OFFICE.

CLARENCE L. DELACHAUX, OF GENNEVILLIERS, FRANCE.

## METHOD OF AND APPARATUS FOR REPAIRING THE ENDS OF RAILS BY THE ALUMINOTHERMIC PROCESS.

Application filed August 15, 1923, Serial No. 657,524, and in France October 30, 1922.

The invention relates to a novel method of and apparatus for repairing the damaged and worn ends of railway rails and, more particularly, the worn tread surfaces of the rails adjacent the joints in the rails caused by the impact of the wheels passing over the breaks in the continuity of the rails at the joints; the worn sections of the rails being restored to their normal condition and contour by means of molten steel applied to such sections by the alumino-thermic welding process, the highly heated molten steel serving to fuse the surfaces of the rail with which it is in contact and to merge and weld therewith to form a substantially homogeneous union, the applied steel being substantially worked to proper shape and contour after it has cooled to a sufficient degree to permit of such operation.

20 The application of the invention is illustrated in the accompanying drawings in which:

Fig. 1 is a side elevation of a typical rail joint illustrating the characteristic wear and impairment of the rail ends due to the passage of the wheels of traffic over the joint.

25 Fig. 2 is a similar view showing the apparatus and the mode of applying the same in repairing and restoring the worn end of one of the rails.

30 Fig. 3 is a transverse vertical section of the same.

It is a well known fact that the ends of railway rails, which are not connected by rigid, welded joints, but are secured together by the usual type of fish plates, splice bars, or the like, are separated by intervals of greater or less width which cause breaks in the continuity of the traction surfaces of 35 treads of the rails which produce decided shocks and jars whenever a wheel passes over the joint. This jarring effect soon becomes sufficiently strong to cause the wheels to rebound and engage the track some distance ahead in the direction of travel with a severe hammer-like blow or concussion, which tends to crush down and wear away the treads of the rails and form depressions, such as indicated at A in Fig. 1. When 40 these depressions become pronounced as to length and depth, they render the track structure dangerous to traffic, especially high speed traffic, and not only hasten the practical destruction of the particular end 45 of the rail, but seriously impair the rolling stock operating thereon and also the road bed. It therefore becomes necessary that these defects be eliminated, which can usually be effected by cutting off the damaged section of the rail, or by replacing the 50 damaged rail by a new one. The first expedient is wholly unsatisfactory, as it means practically removing and readjusting large sections of the track, and the other procedure is prohibitive since it involves the discarding of rails which are unserviceable only in a small fraction of their length, while the remaining portion of the rail is entirely serviceable. It has, therefore, been suggested and attempted heretofore to repair the worn or impaired portions of the rail in situ and without disturbing the track structure. Among the other methods of repair suggested has been that of rebuilding the worn sections or portions of the rail 55 tread by electrically welding steel thereto, but, owing to the uncertainty of electric welded joints of this character, the high degree of skill to produce a satisfactory weld, and the slowness of the electric welding method, the same has been practically discarded as too expensive, if it is to be thoroughly and efficiently applied. The present invention, however, provides a method for rebuilding, restoring and repairing worn or 60 damaged rail sections by the application of highly heated molten steel or the like to the impaired section, by means of the alumino-thermic casting and welding process, which has proven simple and cheap in application 65 and may be carried out by any intelligent workman without special skill or training.

The method aforesaid consists in adjusting and applying to the damaged rail a mold similar to that employed in effecting the 70 alumino-thermic welding of the rail joints, which will enclose the portion of the rail to be repaired and restored. The mold is preferably formed of two sections 4 and 5 divided in a horizontal plane and adapted to be 75 clamped about the portion of the rail to be repaired, as shown in Figs. 2 and 3. The mold cavity proper is preferably of substantially the size and contour of the original rail section, or slightly enlarged as to size to permit of a slight excess of metal being applied to the rail section, which excess is subsequently worked down or machined off to bring the repaired rail into conformity with its original size and contour. In case the rail to 80

85

90

95

100

105

110

be repaired is of the groove type, as illustrated in Fig. 3, the upper section of the mold is provided with a rib 6 which accurately fits the groove in the rail and prevents access of the molten metal to said groove. Connected with the main cavity of the mold is a pouring gate 9, leading to the top of the mold, and a riser 10, these passageways being made relatively much larger, 10 as to volumetric capacity than in ordinary practice, in order to provide a relatively large amount of superheated molten steel, which will have the effect of heating the surfaces of the rail with which it comes in contact sufficiently to cause the same to fuse and to become firmly welded with the steel in the main cavity of the mold. The highly heated molten steel is supplied from a suitable crucible 11, containing an alumino-thermic mixture, which is ignited in the usual way and which produces a molten body 12 of superheated steel, which is delivered from the pouring opening of the crucible into the gate 9, whence the fluid steel passes 20 downward into the main cavity of the mold and into contact with the impaired section of the rail and flows upward into the riser 10, the level of the molten steel in the riser indicating when a sufficient quantity of steel 25 has been supplied to effect the desired purpose. It will be understood, of course, that the amount of superheated molten steel to be supplied will depend largely upon the area and depth of the depression in the rail end 30 to be filled and restored. After the necessary amount of steel has been supplied to effect the proper heating and welding action between the applied steel and the rail surface within the mold cavity, the pouring operation 35 is stopped and the mold allowed to stand until the steel has solidified, after which the upper section of the mold is taken off, and, while the applied steel and the contacting surfaces of the rail are still hot, the steel, 40 which has been applied to the surface of the rail, is forged or worked by means of a sledge, or other suitable means or operation, until it assumes the original form and contour of the rail. This working of the hot 45 steel also has the effect of refining and improving the same and effecting a more complete and homogeneous union between the alumino-thermic steel and the metal of the rail section. The repaired rail is then permitted 50 to cool slowly, and is prevented from chilling unduly by the lower part of the mold, which is permitted to remain in place while the finishing operation, as hereinbefore described, is carried out. If found necessary, the repaired part may be brought to any ultimate desired contour, corresponding 55 with the original form of the rail, by filing or grinding away any surplus metal. Under certain circumstances, it may be found 60 sufficient to permit the applied metal to cool

sufficiently, then remove the entire mold and reduce the applied metal to ultimate form by grinding, without any hammering or swaging or similar operations.

It will usually be found of advantage to 70 preheat the rail section to be repaired before applying the alumino-thermic steel theretc. and this preheating may be effected by enclosing the rail section in the mold, as hereinbefore described, and then directing the flame of an acetylene, oxyhydrogen, or other gas or gasoline torch through the pouring gate into contact with the rail surface within the cavity of the mold. The heat thus applied not only reduces the amount of heat 75 to be furnished by the alumino-thermic steel, and, therefore, the quantity of steel required for the reaction, but also facilitates the successful application of the hot metal by eliminating, at the initiation of the casting operation, the relatively violent reaction between the alumino-thermic steel and the metal of the rail due to the high degree of heat imparted to the relatively cold rail by the superheated steel. By preheating the rail, as indicated, the temperature of the latter is raised gradually and all of the objectionable 80 effects of sudden and violent heating are obviated.

It will also be apparent that, by making 85 additions of suitable metals to the alumino-thermic iron in the crucible, a metal of exactly the same chemical composition as that of the rail ends may be obtained, so that 90 when the repairs to the damaged or impaired sections of the rail have been made, the rail will be restored to its original condition, not only as to contour and shape, but also as to 95 its metallic constituency. For example, 100 suitable additions of carbon, silicon, manganese, chromium, nickel, or titanium may be made to the alumino-thermic mixture, so as to bring the composition of the alumino-thermic additions to the impaired rail into 105 exact consonance with the composition of the original rail. This feature of the 110 method is of particular value and significance in view of the fact that it is extremely difficult to effect electric welding by means of these various steel alloys, because it is not 115 feasible or economical to effect the repairs of damaged rails by the electric welding method on account of the difficulty of forming electrodes of certain of the steel alloys 120 mentioned.

When the method is carried out, as hereinbefore described, it will be obvious that the worn and impaired section of the rail will be restored to its original character, both as to contour and composition, at a minimum 125 of labor and expense.

What I claim is:

1. The method of repairing worn surfaces 130 of rails, which comprises enclosing the rail at the place to be repaired in a mold having

- a cavity of substantially the size and contour of the original rail section, said cavity connecting with a pouring gate and a riser of relatively large size to materially increase 5 the volumetric capacity of the mold, supplying the mold with alumino-thermic steel to fill the cavity and connecting passages with the highly heated molten steel and cause the latter to fuse with the engaging 10 surface of the rail, removing the mold, and working the hot steel application to the desired contour to restore the impaired rail section.
2. The method of repairing worn surfaces of rails, which comprises enclosing the rail at the place to be repaired in a mold having a cavity of substantially the size and contour of the original rail section, said cavity connecting with a pouring gate and a 15 riser of relatively large size to materially increase the volumetric capacity of the mold,
- preliminarily heating the rail at the section to be repaired, supplying the mold with alumino-thermic steel to fill the cavity and connecting passages with the highly-heated 25 molten steel and cause the latter to fuse with the engaging surface of the rail, removing the mold, and working the hot steel application to the desired contour to restore the impaired rail section. 30
3. Means for repairing worn surfaces of rails by alumino-thermic welds, comprising a mold in two separable sections adapted to be clamped about the rail section and having a cavity of substantially the size and 35 contour of the original rail section and a gate and riser of relatively large volumetric capacity to provide a surplus of superheated alumino-thermic metal to heat the surface of the impaired rail section to the fusion point. 40

In testimony whereof I affix my signature.  
C. DELACHAUX.